

# United States Patent

[19]

4,009,029

Hammond et al.

[11]

Feb. 22, 1977

[54] CYANOETHYL-CONTAINING BLOCKED DEVELOPMENT RESTRAINERS

[75] Inventors: Howell Allen Hammond; Wilbert Jeptha Humphlett; Ilmari Fritiof Salminen, all of Rochester, N.Y.

[73] Assignee: Eastman Kodak Company, Rochester, N.Y.

[22] Filed: June 20, 1975

[21] Appl. No.: 588,976

## Related U.S. Application Data

[63] Continuation-in-part of Ser. No. 367,306, June 5, 1973, abandoned.

[52] U.S. Cl. 96/3; 96/29 D; 96/66.3; 96/73; 96/74; 96/76 R; 96/77; 96/95; 96/99; 96/100; 96/109

[51] Int. Cl.<sup>2</sup> G03C 7/00; G03C 5/30; G03C 1/48; G03C 1/40

[58] Field of Search 96/95, 76 R, 77, 3, 96/29 D, 66.3, 109, 73, 74, 99, 100

## References Cited

### UNITED STATES PATENTS

|           |        |                |         |
|-----------|--------|----------------|---------|
| 2,819,965 | 1/1958 | Murray et al.  | 96/109  |
| 2,981,624 | 4/1961 | Dersch et al.  | 96/109  |
| 3,260,597 | 7/1966 | Weyerts et al. | 96/3    |
| 3,265,498 | 8/1966 | Rogers et al.  | 96/3    |
| 3,420,664 | 1/1969 | Dersch et al.  | 96/66.5 |
| 3,632,345 | 1/1972 | Marx et al.    | 96/95   |

|           |         |                  |        |
|-----------|---------|------------------|--------|
| 3,674,478 | 7/1972  | Grasshoff et al. | 96/3   |
| 3,698,897 | 10/1972 | Gompf et al.     | 96/3   |
| 3,756,821 | 9/1973  | Hayashi et al.   | 96/55  |
| 3,785,813 | 1/1974  | Rickter          | 96/3   |
| 3,839,041 | 10/1974 | Hiller           | 96/109 |
| 3,893,859 | 7/1975  | Burness et al.   | 96/109 |

## FOREIGN PATENTS OR APPLICATIONS

768,071 7/1971 Belgium

## OTHER PUBLICATIONS

Allen and Humphlett, "The Thermal Reversibility of . . . Reaction. V", Canadian J. of Chem. vol. 44, 1966, pp. 2315-2321.

Primary Examiner—David Klein

Assistant Examiner—Richard L. Schilling

Attorney, Agent, or Firm—G. E. Battist

## [57] ABSTRACT

Photographic elements are disclosed which contain a blocked development restrainer which is designed to provide timely release of a development restrainer when the photographic element is processed with an alkaline processing composition. The photographic elements are especially useful in image-transfer film units where the blocked development restrainers will permit initial development to occur and, upon cleavage, will substantially restrain further development.

33 Claims, 2 Drawing Figures

### DENSITY OF DEVELOPED SILVER



FIG. 1

## EXPOSED AREA OF PHOTOGRAPHIC ELEMENT

DENSITY OF DEVELOPED SILVER



FIG. 2

DENSITY OF DEVELOPED SILVER

## UNEXPOSED AREA OF PHOTOGRAPHIC ELEMENT



## CYANOETHYL-CONTAINING BLOCKED DEVELOPMENT RESTRAINERS

This application is a continuation-in-part of U.S. Ser. No. 367,306 filed June 5, 1973, now abandoned.

NO. 37,500 filed June 3, 1973, now abandoned.

This invention relates to photographic elements and processes for developing image records in photographic elements. In one aspect, this invention relates to photographic elements which contain development-restrainer precursors. In another aspect, this invention relates to image-transfer photographic film units containing development-restraining precursors.

It is known in the art to use development arrestors and development-arrestor precursors in photographic systems, as mentioned in U.S. Pat. Nos. 3,260,597 by Weyerts et al. and 3,265,498 by Rogers. In these references, the development arrestor was generally made available after a predetermined length of time by positioning it in a receiver layer and/or using a hydrolyzable derivative of the development arrestor whereby the action of the development arrestor would be delayed. However, the compounds available in the art did not generally have the necessary control properties whereby they could be incorporated in the photographic element and still permit the necessary development to take place before functioning in their role as development restrainers or development arrestors. In some instances, a low concentration of a compound which quickly hydrolyzed could be located in the photographic element to serve as an antifoggant where it would, in essence, restrain development of the Dmin and Dmax areas with a sacrifice in maximum density to control the density in the Dmin areas. Other attempts have also been made to provide compounds which have the proper release rate whereby they will become more active at higher temperatures, etc., as mentioned in U.S. Pat. Nos. 3,575,699; 3,649,267 and the like. However, it would be desirable to find improved compounds which have appropriate built-in control whereby they would permit substantial development of a silver halide image layer to occur before the compounds became activated to fulfill their development-restrainer function.

We have now found a class of blocked development restrainers (i.e., development-restrainer precursors) which can be used in photographic elements with improved results when processing the element in an alkaline medium. Generally, the class of blocked development restrainers which can be used in accordance with this invention is represented by the formula:



wherein Z represents the nonmetallic atoms (and bonds) necessary to form a nucleus which completes a 5- or 6-membered heterocyclic ring on said structure, including substituted rings, fused rings and the like, and wherein said heterocyclic ring, taken together with the depicted sulfur atom, provides a silver halide development restrainer upon cleavage from the remainder of the molecule; R is a cyano group; and R<sup>1</sup> and R<sup>2</sup> are preferably each hydrogen atoms, but can be alkyl groups having from 1 to 8 carbon atoms, including substituted alkyl groups, or aryl groups containing from

6 to 12 carbon atoms, including substituted aryl groups, provided that at least one of  $R^1$  and  $R^2$  is hydrogen.

The development restrainer moieties which are released upon cleavage can generally be any of the moieties within the formula limitations which are effective in arresting or restraining silver halide development. However, the structure of the remainder of the molecule is designed to provide for the timely release in the alkaline medium encountered in processing photographic elements, and particularly where the alkaline medium has a pH of about 12 (i.e., 12-14). The blocked development restrainers having a cyano group appear to have superior aging properties in a photographic element compared with other blocked development restrainers.

The improvements obtained with the present class of compounds are quite unexpected since closely related compounds do not provide the same improvements.

The present compounds have certain highly advantageous properties compared with the compounds mentioned in U.S. Pat. No. 3,260,597 and especially closely related 5- $\beta$ -acetyl ethylthio-1-phenyl-1,2,3,4-tetrazole mentioned in column 5 of this reference. The compounds of the present invention provide especially

25 good results when incorporated in the photographic element along with negative silver halide emulsions, whereas many of the compounds of U.S. Pat. No. 3,260,597 appear to react so readily as to require positioning of the compound in the receiver sheet to delay

30 action of the development restrainer on the developing silver halide image record. While the compounds of this invention are preferably used in the photosensitive elements when negative silver halide emulsions are employed, they can also be used in cover sheets or 35 receiver sheets, such as when direct-positive emulsions are employed in the element.

In one embodiment, this invention relates to image-transfer film units comprising:

1. a photosensitive element comprising a support  
40 having thereon at least one layer containing a silver  
halide emulsion having associated therewith an image  
dye-providing material and a blocked development  
restrainer of the above formula,

2. an image-receiving layer and  
45 3. means containing an alkaline processing composition adapted to discharge its contents within said film unit.

In another embodiment, this invention relates to a photographic image-transfer film unit containing at least one layer containing a blue-sensitive silver halide emulsion, at least one layer containing a green-sensitive silver halide emulsion and at least one layer containing a red-sensitive silver halide emulsion, and at least one of said silver halide emulsions having associated therewith a blocked development restrainer of the above formula.

FIGS. 1 and 2 are graphs illustrating the amount of silver formed with respect to time in the development process of Example 1. FIG. 1 shows the infrared density of silver developed in the exposed areas, and FIG. 2 shows the infrared density of silver developed in the unexposed areas (fog), for a control element and an element containing a blocked development restrainer in accordance with this invention.

65 The term "blocked development restrainers" as used herein generally refers to development restrainers which contain a blocking group inactivating or rendering ineffective the development-restrainer capabilities

of the compound. Upon cleavage of the blocking group from the molecule, such as by hydrolysis, etc., the compound can again function as a development restrainer. The blocked development restrainers of this invention have a blocking group designed to provide cleavage in an alkaline medium as encountered in a photographic development process.

Generally, the blocked development restrainers which are useful in accordance with this invention are azoles which cleave in alkaline solution to yield mercaptoazoles which are diffusible in alkaline solution.

The useful compounds generally have the formula:



wherein R, R<sup>1</sup>, R<sup>2</sup> and Z are as defined above. The heterocycle groups formed by Z preferably include groups wherein the heterocyclic atoms (i.e., atoms other than carbon) are members of a single heterocyclic ring, as contrasted with compounds containing fused or condensed heterocyclic rings in which the heterocyclic atoms are members of more than one heterocyclic ring. Typical simple heterocyclic nitrogen compounds include triazoles (e.g., 1,2,4-triazoles, benzotriazoles, etc.), diazoles (e.g., imidazoles, benzimidazoles, etc.), pyrimidines, monoazoles (e.g., benzoxazoles, benzothiazoles, etc.) and the like.

In preferred embodiments, the blocked development restrainers of this invention contain a tetrazole nucleus, and preferably a phenyl-substituted tetrazole nucleus.

A typical useful compound according to this embodiment is as follows:



The blocked development restrainers can be made by methods known in the art, such as by the processes described by Allen and Humphlett, "The Thermal Reversability of the Michael Reaction", *Canadian Journal of Chemistry*, Vol. 44, 1966, pp. 2315-2321; particularly useful procedures are described on pp. 2320 and 2321 in Method B and Method C(iii). As an example of one specific preparation, Compound I can be prepared by reacting 1-phenyl-2-tetrazoline-2-thione with acrylonitrile in glacial acetic acid by Method B. In this procedure for making Compound I, the reaction mixture is maintained at 70°-80° C. for 30 minutes and then boiled for 10 minutes. Most of the solvent is removed under reduced pressure. When residue is allowed to stand overnight, the crude product crystallizes.

The cleavage or blocking of the compounds of this invention appear to function by a reverse Michael reaction. The use of the ethylene linkage separating the group:



from the remainder of the molecule appears to give the necessary resonance structure to provide for timely release of the development-restrainer moiety. Generally, the release of the development restrainer is achieved, in accordance with the present invention, by contact with an alkaline medium, however, it is also possible to aid or achieve cleavage by elevating the temperature, etc.

The release mechanism appears to be different in kind from the release mechanism of compounds such as, for example, the carboxymethylmercapto-substituted heterocyclic nitrogen compounds of U.S. Pat. No. 2,819,965. Generally, the carboxymethylmercapto-substituted compounds require an acid-catalyzed reaction in the presence of a heavy metal salt; this apparently accounts for their usefulness as antifoggants for photographic emulsions subjected to extreme storage conditions.

The photographic elements of this invention can contain the blocked development restrainer in any concentration necessary for the intended purpose, depending on the location of the development restrainer and the problems encountered. In certain embodiments where the blocked development restrainer is associated with a silver halide emulsion layer, the blocked development restrainer can be used at a concentration of at least 0.005 mole/mole of silver in said layer and preferably at a concentration of at least 0.1 mole/mole of silver up to equimolar amounts. In certain embodiments where the compound cleaves to provide a 1-phenylmercaptotetrazole, the blocked development restrainer is preferably used at concentrations of from 0.02 to 0.1 mole/mole of silver. The blocked development restrainer can be incorporated in the photographic element where it is in the layer containing the silver halide emulsion or in an adjacent layer associated therewith. In certain embodiments, the blocked development restrainer is used in association with only one layer of a multiple-layer silver halide element. In still other embodiments, it can be contained in a layer which is placed in intimate contact with the photographic element during processing. The layers of the photographic elements can be hardened during or after coating, as known in the art.

45 In certain embodiments, the blocked development  
restrainers of this invention are incorporated in a cover  
sheet or a receiver element which is in intimate associa-  
tion with the photographic element during processing.  
Cover sheets and receiver elements used for this pur-  
50 pose can have an acid layer, which is used to neutralize  
the pH of the processing composition, with an over-  
coated timing layer which provides for a predetermined  
time for processing before the processing composition  
is neutralized. When the blocked development restrain-  
55 ers are used in this embodiment, they can be coated in  
the timing layer, on top of the timing layer, or behind  
the timing layer, depending upon the amount of time  
desired before the action of the development restrainer  
is desired.

is desired.

60 The blocked development restrainers can be incorporated in the photographic element by dispersing them in the carrier layer by techniques available in the art. In certain preferred embodiments the blocked development restrainers are first dissolved in a high-boiling solvent, such as a water-soluble coupler solvent, and then dispersed in the carrier material. Typical useful coupler solvents are moderately polar solvents such as tri-*o*-cresyl phosphate, di-*n*-butyl phthalate, diethyl-

65

lauramide, 2,4-diamylphenol, liquid dye stabilizers such as described in an article entitled "Improved Photographic Dye Image Stabilizer-Solvent", *Product Licensing Index*, Vol. 83, March, 1971, and the like.

The blocked development restrainers of this invention can generally be used in association with any silver halide emulsion. However, they are preferably used in association with a negative silver halide emulsion, i.e., a silver halide emulsion which develops in the areas of exposure, especially when they are located in close proximity to the silver halide emulsion layers. The silver halide emulsion can have various image dye-providing materials in association therewith to produce in image record with image dyes. Photographic color couplers including compounds as described in U.S. Pat. Nos. 3,046,129 by Graham and 3,620,747 by Mar-  
chant, both incorporated herein by reference, can be used to form the image dye when color developers are used in the process.

The term "image dye-providing material" as used herein is understood to refer to those compounds which either (1) do not require a chemical reaction to form the image dye or (2) undergo reactions encountered in photographic imaging systems to produce an image dye, such as with color couplers, oxichromic compounds and the like. The first class of compounds is generally referred to as preformed image dyes and includes shifted dyes, etc., while the second class of compounds is generally referred to as dye precursors.

The terms "initially diffusible" and "initially immobile" as used herein refer to compounds which are incorporated in the photographic element and, upon contact with an alkaline processing solution, are substantially diffusible or substantially immobile, respectively.

The image dye-providing materials in one preferred embodiment where negative silver halide emulsions are used, can be initially mobile image dye-providing materials such as those used in image-transfer photographic elements. Typical useful, initially mobile image dye-providing materials include dye developers as disclosed in U.S. Pat. Nos. 2,983,606; 3,255,001 and the like; oxichromic developers which undergo chromogenic oxidation to form image dyes as disclosed in U.S. Ser. No. 308,869 filed Nov. 22, 1972, now U.S. Pat. No. 3,880,658 issued Apr. 29, 1975; shifted indophenol dye developers as disclosed in U.S. Pat. No. 3,854,945 by Bush and Reardon issued Dec. 17, 1974; metalized dye developers as disclosed in U.S. Pat. Nos. 3,482,972; 3,544,545; 3,551,406 and 3,563,739; and the like: all of which are incorporated herein by reference.

The image dye-providing material in another preferred embodiment, especially when negative silver halide emulsions are used, is an initially immobile image dye-providing material. Preferably, the initially immobile image dye-providing material is a positive-working immobile photographic compound such as disclosed in Hinshaw and Condit, U.S. Ser. No. 326,628 filed January 26, 1973, which is incorporated herein by reference.

In another embodiment, immobile image dye-providing compounds can be used in association with silver halide emulsions wherein said compounds undergo oxidation followed by hydrolysis to provide an image-wise distribution of a mobile image dye. Compounds of this type can be used with negative emulsions to form positive image records in the exposed photographic

element, or they can be used with direct-positive or reversal emulsions to form positive transfer images such as in an image-transfer film unit. Typical useful immobile image dye-providing compounds are disclosed in Canadian Pat. No. 602,607 by Whitmore et al. issued Aug. 2, 1960, U.S. Ser. Nos. 351,673 by Fleckenstein et al. published as trial voluntary protest No. B 351,673 on Jan. 28, 1975 and 351,700 by Fleckenstein issued as U.S. Pat. No. 3,928,312 on Dec. 13, 1975, and U.S. Pat. Nos. 3,698,897 by Gompf et al., 3,728,113 by Becker et al., 3,725,062 by Anderson et al., 3,227,552 by Whitmore, 3,443,939; 3,443,940 and 3,443,941, and the like, all of which are incorporated herein by reference.

In still other embodiments, the blocked development restrainers can be used in photographic elements containing a layer comprising a negative silver halide emulsion and having an adjacent layer containing physical development nuclei associated with an image dye-providing material. Typical photographic elements of this type are disclosed in U.S. Pat. No. 3,227,551 (col. 6 and 7) and British Pat. No. 904,364 (p. 19), which are incorporated herein by reference.

The silver halide emulsions used in the photographic elements of this invention can comprise silver chloride, silver bromide, silver bromoiodide, silver chlorobromoiodide and the like, or mixtures thereof. The emulsions may be coarse- or fine-grain and can be prepared by any of the well-known procedures, e.g., single-jet emulsions, double-jet emulsions, such as Lippmann emulsions, ammoniacal emulsions, thiocyanate or thioether ripened emulsions such as those described in U.S. Pat. Nos. 2,222,264 by Nietz et al., 3,320,069 by Illingsworth and 3,271,157 by McBride. Surface-image emulsions can be used or internal-image emulsions can be used such as those described in U.S. Pat. Nos. 2,592,250 by Davey et al., 3,206,313 by Porter et al. and 3,447,927 by Bacon et al. The emulsions may be regular-grain emulsions such as the type described in Klein and Moisar, *J. Phot. Sci.*, Vol. 12, No. 5, September/October, 1964, pp. 242-251. If desired, mixtures of surface- and internal-image emulsions can be used as described in Luckey et al., U.S. Pat. No. 2,996,382.

Negative-type emulsions can be used or direct-positive emulsions can be used such as those described in U.S. Pat. Nos. 2,184,013 by Leermakers, 2,541,472 by Kendall et al., 3,367,778 by Berriman, 3,501,307 by Illingsworth et al. issued Mar. 17, 1970, 2,563,785 by Ives, 2,456,953 by Knott et al., 2,861,885 by Land, 3,761,276 by Evans, 3,761,266 by Milton, 3,761,267 by Gilman et al., 3,736,140 by Collier et al., and 3,730,723 by Gilman et al., U.S. Ser. No. 154,155 by Gilman et al. filed June 17, 1971, now abandoned, and British Pat. No. 723,019 by Schouwenaars.

The blocked development restrainers in accordance with this invention are preferably used in photographic elements designed for one-step processing or processing with a single alkaline liquid composition. The development of the silver halide layers can proceed for a specified period with timely hydrolysis of the compound to provide a development restrainer which assists in shutting down further development and preventing interaction of reactants with the wrong silver halide layer.

In certain preferred embodiments, the blocked development restrainers are used in the photographic element of an image-transfer film unit. The photographic element can be used in image-transfer film units as

described, for example, in U.S. Pat. Nos. 2,543,181; 2,983,606; 3,227,550; 3,227,552; 3,415,645; 3,415,644; 3,415,646 and 3,635,707, Canadian Pat. No. 674,082, and Belgian Pat. Nos. 757,959 and 757,960, both issued Apr. 23, 1971. In highly preferred embodiments, the blocked development restrainers are used in the photographic element of an image-transfer film unit which is designed to be processed with a single processing solution, and the resulting positive image is viewed through a transparent support and against an opaque background.

The blocked development restrainers of this invention are advantageously used in image-transfer elements wherein it is desired to allow development to occur for a predetermined period of time, followed by inhibition of further development. The blocked development restrainers are generally useful in image-transfer film units which comprise:

1. a photosensitive element comprising a support having thereon at least one layer containing a silver halide emulsion having associated therewith an image dye-providing material and preferably at least three layers which contain, respectively, a blue-sensitive silver halide emulsion, a green-sensitive silver halide emulsion and a red-sensitive silver halide emulsion;

2. an image-receiving layer which can be located on a separate support and superposed on said support containing said silver halide emulsions layers or, preferably, it can be coated on the same support adjacent to the photosensitive silver halide emulsion layers; and

3. means containing an alkaline processing composition adapted to discharge its contents within said film unit.

Where the receiver layer is coated on the same support with the photosensitive silver halide layers, the support is preferably a transparent support, an opaque layer is preferably positioned between the image-receiving layer and the photosensitive silver halide layer, and the alkaline processing composition preferably contains an opacifying substance such as carbon or a pH-indicator dye which is discharged into the film unit between a dimensionally stable support or cover sheet and the photosensitive element.

In certain embodiments, the cover sheet can be superposed or adapted to be superposed on the photosensitive element. The image-receiving layer can be located on the cover sheet. In certain preferred embodiments where the image-receiving layer is located in the photosensitive element, a neutralizing layer is located

5 point of desired discharge of its contents into the film unit and adapted to be passed between a pair of juxtaposed rollers to effect discharge of the contents into the film unit, frangible containers positioned over or within the photosensitive element, hypodermic syringes, and the like.

10 It is known in the art that neutralizing layers containing acidic materials, such as polymeric acids, monomeric acids, hydrolyzable materials and the like, can be positioned within an image-transfer film unit to effect shutdown of development of silver halide and transfer of the image dye-providing substance. Neutralizing layers can also be used in the film units of the present invention, including acid layers positioned behind timing layers to delay neutralization of the element, acid layers positioned near the image-receiving layer, acid layers on a cover sheet used to distribute the processing composition uniformly over the photosensitive element, acid layers within the photosensitive element, and the like. However, since most image dye-providing materials transfer at much higher rates in a highly alkaline medium than in a neutral medium, it is desirable to delay neutralization until after the image dye-providing material has completed the necessary transfer. It is 15 apparent that the image dye-providing materials will transfer through adjacent silver halide layers in an environment wherein interactions can still occur. The blocked development restrainers of this invention can be used effectively to reduce the interactions of diffusible material with the adjacent layers to prevent contamination and still allow the film unit to be maintained in a highly alkaline medium for sufficient time to achieve high densities of transferred image dye-providing material.

20 25 30 35 40 The invention can be further demonstrated by the following examples.

Examples 1-3 demonstrate a preferred embodiment wherein the blocked development restrainers are used in a photographic element containing a negative silver halide emulsion having associated therewith an initially diffusible oxichromic compound. Example 1 also shows comparisons with prior-art compounds.

#### EXAMPLE 1

45 A photographic element is prepared by coating layers in order on a support as follows:

1. transparent support;
2. layer containing 125 mg./ft.<sup>2</sup> of gelatin and 35 mg./ft.<sup>2</sup> of the oxichromic developer:



65 on the cover sheet.

A means for containing the alkaline processing solution can be any means known in the art for this purpose, including rupturable containers positioned at the

dissolved in diethyl lauramide at 24 mg./ft.<sup>2</sup>;

65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 973

of 1-phenyl-3-pyrazolidone, and 0.79 millimole/ft.<sup>2</sup> of the hydrolyzable development restrainer per Table 1; 4. layer containing 70 mg./ft.<sup>2</sup> of gelatin;

Samples of the elements are evaluated for the amount and rate of silver developed in the photographic silver halide negative (Procedure A) and the transferred dye image and developed silver after a 30-second transfer process (Procedure B).

#### Procedure A

An infrared reflectance densitometer is used to monitor the silver development as a function of time. This is achieved by measuring the development of silver through the transparent support of an unexposed sample (fog development) and a sample which has been light-flashed (image development). Development is

#### Procedure B

To evaluate the transferred dye image and developed silver of the above prepared elements, separate samples are exposed through a graduated-density test object and activated with a viscous solution having 65 g./l. potassium hydroxide and 30 g./l. hydroxyethyl cellulose while in contact with a receiving element comprising a supported layer of the dye mordant octadecyl tributylammonium bromide (200 mg./ft.<sup>2</sup>) in di-n-butylphthalate (200 mg./ft.<sup>2</sup>) and gelatin (700 mg./ft.<sup>2</sup>). After 30 sec., the receiver is separated from the negative element. The amount of developed silver is measured after the 30-sec. transfer period and is recorded in Table 1. The resulting image density on the receiver is measured and is also recorded in Table 1.

Table 1

| Compound                                                                | Procedure A                    |           | Procedure B                  |                  | Silver (mg.) Dev. on Negative |                  |
|-------------------------------------------------------------------------|--------------------------------|-----------|------------------------------|------------------|-------------------------------|------------------|
|                                                                         | IR Density of Developed Silver |           | Dye Den-<br>sity on Receiver |                  | D <sub>max</sub>              | D <sub>min</sub> |
|                                                                         | Exposed                        | Unexposed | D <sub>max</sub>             | D <sub>min</sub> |                               |                  |
| phenylmer-<br>captotetra-<br>azole*                                     | 76                             | 1         | 1.79                         | 1.33             | 9                             | 2                |
| none<br>(control)                                                       | 97                             | 75        | 1.46                         | .13              | 24                            | 8                |
| I**                                                                     | 90                             | 18        | 1.68                         | .13              | 14                            | 1                |
| none<br>(control)                                                       | 98                             | 77        | 1.64                         | .13              | 24                            | 3                |
| 5- $\beta$ -acetyl-<br>ethylthio-<br>1-phenyl-<br>1,2,3,4-<br>tetrazole | 7                              | 0         | 1.83                         | 1.78             | 2                             | 0                |
| none<br>(control)                                                       | 98                             | 65        | 1.64                         | .13              | 19                            | 2                |

\*.0079 mmole/ft.<sup>2</sup>

\*\*Compound I = 5-(2 cyanethylthio)-1 phenyltetrazole which is a compound of the invention.

accomplished by spreading a viscous activating solution having 40 g./l. potassium hydroxide and 30 g./l. 40 hydroxyethyl cellulose.

The data from the above Table 1 are then standardized to a single control. They are recorded in Table 2 below.

Table 2

| Compound                                                                | Procedure A                        |           | Procedure B      |                  | Dev. Silver (mg.) |                  |
|-------------------------------------------------------------------------|------------------------------------|-----------|------------------|------------------|-------------------|------------------|
|                                                                         | IR of Density of Total Silver Dev. |           | Dye Dens.        |                  | D <sub>max</sub>  | D <sub>min</sub> |
|                                                                         | Exposed                            | Unexposed | D <sub>max</sub> | D <sub>min</sub> |                   |                  |
| none (control)                                                          | 98                                 | 77        | 1.64             | .13              | 24                | 3                |
| phenylmer-<br>captotetra-<br>azole                                      | 76                                 | 1         | 2.0              | 1.3              | 9                 | .8               |
| I                                                                       | 88                                 | 15        | 1.70             | .13              | 14                | 0.9              |
| 5- $\beta$ -acetyl-<br>ethylthio-<br>1-phenyl-<br>1,2,3,4-<br>tetrazole | 7                                  | 0         | 1.83             | 1.78             | 3                 | 0                |

The unexposed sample is monitored for times up to 5 min., and the exposed sample is monitored for 14 sec. This procedure gives data which are illustrated for one of the compounds of the invention as compared with a control which does not contain the blocked development restrainer by FIG. 1 and 2. The total silver density developed in both the exposed (14-sec. development time) and the unexposed (5-min. development time) samples is recorded in Table 1.

From the data listed in Tables 1 and 2, one can observe that the compounds of the invention are effective in reducing silver development in the unexposed sample without substantially affecting development in the exposed sample (Procedure A). The data from Procedure B illustrate that increased maximum dye density is obtained without increasing density in the fully exposed regions, i.e., D<sub>min</sub>. This is explained by the fact that upon activation the oxichromic developer in Layer 2 is solubilized and begins to diffuse to the receiver. The

developing silver in Layer 3 causes the imagewise immobilization of the compound by oxidation. The 1-phenyl-3-pyrazolidone contained in Layer 3 acts as an auxiliary developer to aid in imagewise oxidation. If the silver halide emulsion in Layer 3 develops in the unexposed areas before all the diffusible oxichromic compound has migrated to the receiver, it will cause a loss in maximum dye density. Further, if the development of image silver has been inhibited, it will not be effective in immobilizing the oxichromic dye compound, and undesirable dye will transfer in areas of maximum exposure, as exhibited by the 5-B-acetylethylthio-1-phenyl-1,2,3,4-tetrazole which apparently hydrolyzes so quickly that development is substantially inhibited.

## EXAMPLE 2

An integral color transfer photographic element is prepared as follows (the full identification of certain components follows the example):

1. transparent polyethylene terephthalate support; 20
2. dye mordant layer containing gelatin at 100 mg./ft.<sup>2</sup> and copoly[styrene-N-benzyl-N,N-dimethyl-N-(3-maleimidopropyl)ammonium chloride] at 200 mg./ft.<sup>2</sup>;
3. layer containing titanium dioxide at 2000 mg./ft.<sup>2</sup> and gelatin at 200 mg./ft.<sup>2</sup>;
4. layer containing carbon opacifying agent at 250 mg./ft.<sup>2</sup> and gelatin at 156 mg./ft.<sup>2</sup>;
5. layer containing gelatin at 75 mg./ft.<sup>2</sup>, 2,5-disec-dodecylhydroquinone at 70 mg./ft.<sup>2</sup> and tricresyl phosphate at 23 mg./ft.<sup>2</sup>; 30
6. layer containing a red-sensitive silver bromoiodide emulsion at 80 mg./ft.<sup>2</sup> based on silver, gelatin at 82 mg./ft.<sup>2</sup>, OC-I at 43 mg./ft.<sup>2</sup> dissolved in diethyl lauramide at 29 mg./ft.<sup>2</sup>, and 4-methylphenyl hydroquinone at 15 mg./ft.<sup>2</sup>;
7. layer containing gelatin at 150 mg./ft.<sup>2</sup>, 2,5-disec-dodecylhydroquinone at 70 mg./ft.<sup>2</sup> and a magenta filter dye at 30 mg./ft.<sup>2</sup> dissolved in diethyl lauramide at 50 mg./ft.<sup>2</sup>; 40
8. layer containing a green-sensitive silver bromoiodide emulsion at 80 mg./ft.<sup>2</sup> based on silver, gelatin at 102 mg./ft.<sup>2</sup>, OC-III at 63 mg./ft.<sup>2</sup> dissolved in diethyl lauramide at 39 mg./ft.<sup>2</sup>, and 4-methylphenyl hydroquinone at 15 mg./ft.<sup>2</sup>;
9. layer containing gelatin at 150 mg./ft.<sup>2</sup>, 2,5-disec-dodecylhydroquinone at 70 mg./ft.<sup>2</sup> and a yellow filter dye at 100 mg./ft.<sup>2</sup> dissolved in diethyl lauramide at 28 mg./ft.<sup>2</sup>; 50
10. layer containing a blue-sensitive silver bromoiodide emulsion at 100 mg./ft.<sup>2</sup> based on silver, gelatin at

124 mg./ft.<sup>2</sup>, OC-II at 73 mg./ft.<sup>2</sup> dissolved in diethyl lauramide at 44 mg./ft.<sup>2</sup>, and 4-methylphenyl hydroquinone at 15 mg./ft.<sup>2</sup>;

11. layer containing gelatin at 50 mg./ft.<sup>2</sup>.

A transparent cover sheet for the above element is prepared as follows:

1. transparent polyethylene terephthalate support;
2. layer containing gelatin at 900 mg./ft.<sup>2</sup>, polyacrylic acid at 900 mg./ft.<sup>2</sup> and imidazole at 760 mg./ft.<sup>2</sup>;
3. layer containing cellulose acetate at 1140 mg./ft.<sup>2</sup> and copoly(styrene-maleic anhydride) at 60 mg./ft.<sup>2</sup>.

The photographic element is exposed through a multicolor graduated-density test object, the transparent cover sheet superposed on the element, and a pod containing an opaque processing composition is ruptured to discharge between the cover sheet and the photosensitive element by passing the film unit through juxtaposed rollers having a gap of about 8 mils.

The processing composition is as follows:

|                                    |          |
|------------------------------------|----------|
| potassium hydroxide                | 40 g./l. |
| hydroxyethyl cellulose             | 25 g./l. |
| potassium bromide                  | 80 g./l. |
| $\alpha$ -benzylpicolinium bromide | 10 g./l. |
| bis-methylsulfonmethane            | 2 g./l.  |
| carbon                             | 40 g./l. |
| water to 1 liter                   |          |

After 4 min., the backing sheet is separated from the exposed element and the element is immersed in a 2% sodium persulfate bath for 1 min., washed for 10 min., and dried.

The samples processed are as follows:

|            |                                                                                                                                                         |
|------------|---------------------------------------------------------------------------------------------------------------------------------------------------------|
| Element 1: | control (as above)                                                                                                                                      |
| Element 2: | same as control except each of Layers 7 and 9 contains 5 mg./ft. <sup>2</sup> of Compound I dissolved in 15 mg./ft. <sup>2</sup> of tricresyl phosphate |
| Element 3: | same as control except each of Layers 6 and 8 contains 5 mg./ft. <sup>2</sup> of Compound I dissolved in 15 mg./ft. <sup>2</sup> of tricresyl phosphate |

Table 3

| Element | $D_{max}$ |       |      | $D_{min}$ |       |      |
|---------|-----------|-------|------|-----------|-------|------|
|         | Red       | Green | Blue | Red       | Green | Blue |
| 1       | 0.56      | 0.78  | 1.18 | 0.24      | 0.32  | 0.36 |
| 2       | 1.37      | 1.71  | 2.15 | 0.22      | 0.24  | 0.35 |
| 3       | 1.52      | 1.81  | 2.20 | 0.22      | 0.26  | 0.36 |

OC-II is:



OC-III is:

-continued



OC-I is the oxichromic developer used in Example 1, Layer 2.

The oxichromic compounds used in this example and the following examples can be prepared as described in Lestina and Bush, U.S. Ser. No. 308,869 filed Nov. 22, 1972.

### EXAMPLE 3

An integral color transfer photographic element is prepared as follows (the full identification of certain components follows the example):

1. transparent polyethylene terephthalate support;
2. dye mordant layer containing gelatin at 100 mg./ft.<sup>2</sup>, copoly[styrene/N-benzyl-N,N-dimethyl-N-(3-maleimidopropyl)-ammonium chloride] at 200 mg./ft.<sup>2</sup> and a nitroxyl oxidant at 200 mg./ft.<sup>2</sup>;
3. layer containing titanium dioxide at 2000 mg./ft.<sup>2</sup> and gelatin at 200 mg./ft.<sup>2</sup>;
4. layer containing carbon opacifying agent at 250 mg./ft.<sup>2</sup> and gelatin at 156 mg./ft.<sup>2</sup>;
5. layer containing gelatin at 75 mg./ft.<sup>2</sup>, 2,5-di-sec-dodecylhydroquinone at 70 mg./ft.<sup>2</sup> and tricresyl phosphate at 23 mg./ft.<sup>2</sup>;
6. layer containing a red-sensitive silver bromoiodide emulsion at 70 mg./ft.<sup>2</sup> based on silver, gelatin at 230 mg./ft.<sup>2</sup>, OC-IV at 42 mg./ft.<sup>2</sup> dissolved in 2-cyanoethyl-thio)-lauramide at 73 mg./ft.<sup>2</sup>, 5-(2:cyanoethylthio)-1-phenyltetrazole at 5 mg./ft.<sup>2</sup> dissolved in tricresyl phosphate at 15 mg./ft.<sup>2</sup> and 5,6,7,8-tetrahydro-5,8-methano-1,4-naphthalenediol at 10 mg./ft.<sup>2</sup>;
7. layer containing gelatin at 300 mg./ft.<sup>2</sup>, 2,5-di-sec-dodecylhydroquinone at 70 mg./ft.<sup>2</sup> and a magenta filter dye at 30 mg./ft.<sup>2</sup> dissolved in diethyl lauramide at 50 mg./ft.<sup>2</sup>;
8. layer containing green-sensitive silver bromoiodide emulsion at 70 mg./ft.<sup>2</sup> based on silver, gelatin at 230 mg./ft.<sup>2</sup>, OC-V at 54 mg./ft.<sup>2</sup> dissolved in diethyl lauramide at 64 mg./ft.<sup>2</sup>, 5-(2-cyanoethylthio)-1-phenyltetrazole at 5 mg./ft.<sup>2</sup> dissolved in tricresyl phosphate at 15 mg./ft.<sup>2</sup> and 5,6,7,8-tetrahydro-5,8-methano-1,4-naphthalenediol at 10 mg./ft.<sup>2</sup>;
9. layer containing gelatin at 300 mg./ft.<sup>2</sup>, 2,5-di-sec-dodecylhydroquinone at 70 mg./ft.<sup>2</sup> and a yellow filter dye at 100 mg./ft.<sup>2</sup> dissolved in diethyl lauramide at 28 mg./ft.<sup>2</sup>;
10. layer containing a blue-sensitive silver bromoiodide emulsion at 70 mg./ft.<sup>2</sup> based on silver, gelatin at 210 mg./ft.<sup>2</sup>, OC-VI at 64 mg./ft.<sup>2</sup> dissolved in diethyl

20 lauramide at 106 mg./ft.<sup>2</sup>, 5-(2-cyanoethylthio)-1-phenyltetrazole at 5 mg./ft.<sup>2</sup> dissolved in tricresyl phosphate at 15 mg./ft.<sup>2</sup> and 5,6,7,8-tetrahydro-5,8-methano-1,4-naphthalenediol at 10 mg./ft.<sup>2</sup>;

11. layer containing gelatin at 50 mg./ft.<sup>2</sup>.

A transparent cover sheet for the above element is prepared as follows:

1. transparent polyethylene terephthalate support;
2. layer containing gelatin at 900 mg./ft.<sup>2</sup>, polyacrylic acid at 900 mg./ft.<sup>2</sup> and imidazole at 760 mg./ft.<sup>2</sup>;
3. layer containing cellulose acetate at 1140 mg./ft.<sup>2</sup> and copoly(styrene-maleic anhydride) at 60 mg./ft.<sup>2</sup>.

The photographic element is exposed through a multi-color, graduated-density test object, the transparent cover sheet superposed on the element, and a pod containing an opaque processing composition is ruptured to discharge between the cover sheet and the photosensitive element by passing the film unit through juxtaposed rollers having a gap of about 8 mils.

40 The processing composition is as follows:

|                                                    |          |
|----------------------------------------------------|----------|
| potassium hydroxide                                | 51 g./l. |
| hydroxyethyl cellulose                             | 30 g./l. |
| potassium bromide                                  | 40 g./l. |
| $\alpha$ -benzylpicolinium bromide                 | 15 g./l. |
| 5,6,7,8-tetrahydro-5,8-methano-1,4-naphthalenediol | 15 g./l. |
| carbon                                             | 40 g./l. |

50 After about 1 to 2 min. a well-defined color image with excellent color reproduction is viewed through the transparent support of the integral element.

The nitroxyl oxidant is the compound:



65 The nitroxyl oxidant can be made by reacting the respective ballasted acyl chloride with the 4-amino-2,2,6,6-tetramethylpiperidine-1-oxyl.



Examples 4 and 5 demonstrate a preferred embodiment wherein the blocked development restrainers are used in a photographic element containing a negative silver halide emulsion having associated therewith positive-working, initially immobile, dye-releasing compounds.

#### EXAMPLE 4

A multicolor photographic element is prepared by coating a photographic film support with the following layers in order from the support:

1. layer containing a red-sensitive negative silver halide emulsion (1.2  $\mu$  average grain AgBr) at 150 mg. silver/ft.<sup>2</sup>, gelatin at 170 mg./ft.<sup>2</sup>, Dye Releaser I at 60 mg./ft.<sup>2</sup> dissolved in diethyl lauramide at 30 mg./ft.<sup>2</sup>, 1-phenyl-3-pyrazolidone at 15 mg./ft.<sup>2</sup>, and 5-(2-cyanoethylthio)-1-phenyltetrazole at 12 mg./ft.<sup>2</sup> dissolved in tricresyl phosphate at 36 mg./ft.<sup>2</sup>;

2. layer containing gelatin at 70 mg./ft.<sup>2</sup> and 2,5-di-sec-dodecylhydroquinone at 70 mg./ft.<sup>2</sup> dissolved in diethyl lauramide at 23 mg./ft.<sup>2</sup>;

3. layer containing a green-sensitive negative silver halide emulsion (1.2  $\mu$  average grain AgBr) at 150 mg. silver/ft.<sup>2</sup>, gelatin at 170 mg./ft.<sup>2</sup>, Dye Releaser II at 45 mg./ft.<sup>2</sup> dissolved in diethyl lauramide at 23 mg./ft.<sup>2</sup>,

45 1-phenyl-3-pyrazolidone at 15 mg./ft.<sup>2</sup>, and 5-(2-cyanoethylthio)-1-phenyltetrazole at 12 mg./ft.<sup>2</sup> dissolved in tricresyl phosphate at 36 mg./ft.<sup>2</sup>;

4. layer containing gelatin at 70 mg./ft.<sup>2</sup>, 2,5-di-sec-dodecylhydroquinone at 70 mg./ft.<sup>2</sup> dissolved in diethyl lauramide at 23 mg./ft.<sup>2</sup>, and Carey Lea silver at 17 mg./ft.<sup>2</sup>;

5. layer containing a blue-sensitive negative silver halide emulsion (1.2  $\mu$  average grain AgBr) at 150 mg./ft.<sup>2</sup>, gelatin at 170 mg./ft.<sup>2</sup>, Dye Releaser III at 70 mg./ft.<sup>2</sup> dissolved in diethyl lauramide at 35 mg./ft.<sup>2</sup>, 1-phenyl-3-pyrazolidone at 15 mg./ft.<sup>2</sup>, and 5-(2-cyanoethylthio)-1-phenyltetrazole at 12 mg./ft.<sup>2</sup> dissolved in tricresyl phosphate at 36 mg./ft.<sup>2</sup>;

6. layer containing gelatin at 50 mg./ft.<sup>2</sup>. The photographic element is exposed to a multicolor, graduated-density test object and processed at room temperature with a various aqueous solution comprising 50 g. potassium hydroxide and 30 g. hydroxyethyl cellulose/1. of water, while in contact with a mordanted receiver comprising a polyethylene-coated paper support coated with a layer containing copoly[styrene-N-benzyl-N,N-dimethyl-N-(3-maleimidopropyl)ammonium chloride] at 200 mg./ft.<sup>2</sup> and gelatin at 200

mg./ft.<sup>2</sup> and overcoated with a layer containing 50 mg./ft.<sup>2</sup> gelatin.

Upon separation of the photographic element from the receiver, the receiver is washed, and a well-defined multicolor reproduction of the test object is obtained.

The compounds referred to in this example and the following example are as follows:



monium chloride] at 200 mg./ft.<sup>2</sup> and gelatin at 100 mg./ft.<sup>2</sup>;

2. layer containing titanium dioxide at 2000 mg./ft.<sup>2</sup> and gelatin at 200 mg./ft.<sup>2</sup>;

3. layer containing carbon at 250 mg./ft.<sup>2</sup> and gelatin at 156 mg./ft.<sup>2</sup>;

4. layer containing a red-sensitive negative silver



The dye-releaser compounds can be prepared as generally described in Hinshaw and Condit, U.S. Ser. No. 326,628 filed Jan. 26, 1973.

#### EXAMPLE 5

An integral color transfer photographic element is prepared by coating a transparent film support with the following layers in order from the support:

1. layer containing the mordant copoly[styrene-N-benzyl-N,N-dimethyl-N-(3-maleimidopropyl)am-

halide emulsion (1.2  $\mu$  average grain AgBr) at 150 mg. silver/ft.<sup>2</sup> gelatin at 170 mg./ft.<sup>2</sup>, Dye releaser I at 60 mg./ft.<sup>2</sup> dissolved in diethyl lauramide at 30 mg./ft.<sup>2</sup>, 1-phenyl-3-pyrazolidone at 15 mg./ft.<sup>2</sup>, and 5-(2-cyanoethylthio)-1-phenyltetrazole at 12 mg./ft.<sup>2</sup> dissolved in tricresyl phosphate at 36 mg./ft.<sup>2</sup>;

5. layer containing gelatin at 70 mg./ft.<sup>2</sup> and 2,5-di-secododecylhydroquinone at 70 mg./ft.<sup>2</sup> dissolved in diethyl lauramide at 23 mg./ft.<sup>2</sup>;

6. layer containing a green-sensitive negative silver halide emulsion (1.2  $\mu$  average grain AgBr) at 150 mg.

silver/ft.<sup>2</sup>, gelatin at 170 mg./ft.<sup>2</sup>, Dye Releaser II at 45 mg./ft.<sup>2</sup> dissolved in diethyl lauramide at 23 mg./ft.<sup>2</sup>, 1-phenyl-3-pyrazolidone at 15 mg./ft.<sup>2</sup>, and 5-(2-cyanoethylthio)-1-phenyltetrazole at 12 mg./ft.<sup>2</sup> dissolved in tricresyl phosphate at 36 mg./ft.<sup>2</sup>;

7. layer containing gelatin at 70 mg./ft.<sup>2</sup>, 2,5-di-sec-dodecylhydroquinone at 70 mg./ft.<sup>2</sup> dissolved in diethyl lauramide at 23 mg./ft.<sup>2</sup>, and Carey Lea silver at 17 mg./ft.<sup>2</sup>;

8. layer containing a blue-sensitive negative silver halide emulsion (1.2  $\mu$  average grain AgBr) at 150 mg./ft.<sup>2</sup>, gelatin at 170 mg./ft.<sup>2</sup>, Dye Releaser III at 70 mg./ft.<sup>2</sup> dissolved in diethyl lauramide at 35 mg./ft.<sup>2</sup>, 1-phenyl-3-pyrazolidone at 15 mg./ft.<sup>2</sup>, and 5-(2-cyanoethylthio)-1-phenyltetrazole at 12 mg./ft.<sup>2</sup> dissolved in tricresyl phosphate at 36 mg./ft.<sup>2</sup>;

9. layer containing gelatin at 50 mg./ft.<sup>2</sup>.

The photographic element is exposed to a multicolor graduated-density test object and processed at room temperature by rupturing a pod containing a viscous solution comprising 100 g. potassium hydroxide and 30 g. hydroxyethyl cellulose/1. of water between the photographic element and an opaque cover sheet with a good three-color image appearing in the receiving layer.

#### EXAMPLE 6

The development restrainers can be used in processing cover sheets which are in intimate contact with the photographic element during processing.

Processing cover sheets are prepared as follows:

#### Cover Sheet A (control)

A transparent polyethylene terephthalate support is coated in sequence with a neutralizing layer of poly(butyl acrylate-co-acrylic acid) (30/70 by weight) at 21.5 mg./m.<sup>2</sup> and then a timing layer of a 95/5 mixture of cellulose acetate (40% acetyl) and poly(styrene-co-maleic anhydride) at 4.3 g./m.<sup>2</sup>.

#### Cover Sheet B

A cover sheet is prepared identical to Cover Sheet A except that the timing layer additionally contains 0.11 g./m.<sup>2</sup> of Compound I.

Each cover sheet is then used in processing an integral multicolor photosensitive element prepared by coating the following layers in the order given on a poly(ethylene terephthalate) film support (coverages in parentheses in g./m.<sup>2</sup> unless indicated otherwise):

1. image-receiving layer of poly(styrene-co-N-vinylbenzyl-N,N,N-trihexylammonium chloride) (2.2) and gelatin (2.2);

2. reflecting layer of titanium dioxide (21.5) and gelatin (2.2);

3. opaque layer of carbon black (2.7) and gelatin (1.7);

4. Compound A (0.54) dispersed in gelatin (0.73);

5. red-sensitive, direct-positive, internal-image gelatin-silver bromide emulsion (1.1 Ag, 1.1 gelatin), 5-sec-octadecylhydroquinone-2-sulfonic acid (8.0 g./mole silver), and fogging agent Compound D (1.5 g./mole silver);

6. interlayer of gelatin (0.54) and 2,5-di-sec-dodecylhydroquinone (1.1);

7. Compound B (0.65) dispersed in gelatin (1.05);

8. green-sensitive, direct-positive, internal-image gelatin-silver bromide emulsion (1.1 silver, 1.16 gelatin), 5-sec-octadecylhydroquinone-2-sulfonic acid (16.0 g./mole silver), and fogging agent Compound D (1.5 g./mole silver);

9. interlayer of gelatin (0.54) and 2,5-di-sec-dodecylhydroquinone (1.1);

10. Compound C (1.1) and gelatin (1.1);

11. blue-sensitive, direct-positive, internal-image gelatin-silver bromide emulsion (1.1 silver, 1.1 gelatin), 5-sec-octadecylhydroquinone-2-sulfonic acid (8.0 g./mole silver), and fogging agent Compound D (1.5 g./mole silver);

12. overcoat layer of gelatin (0.54) and hardener bis-(vinylsulfonylmethyl)ether (57.0 mg./m.<sup>2</sup>).

#### Compound Identification



-continued



The photosensitive element is exposed to a tungsten light source through a graduated multicolor test object. The processing composition described below is employed in a pod and is spread between the photosensitive element and each sample of the above cover sheets by passing the transfer "sandwich" between a pair of juxtaposed rollers so that the liquid layer is about 70  $\mu\text{m}$ . in thickness. Comparisons of the cover sheets are made at 15°, 22° and 38° C.

-continued

|    |                                                | <u>Processing Composition</u> |        |
|----|------------------------------------------------|-------------------------------|--------|
| 60 | 4-hydroxymethyl-4-methyl-1-phenyl-3-pyrazolone |                               | 12 g.  |
|    | 5-methylbenzotriazole                          |                               | 4 g.   |
|    | t-butylhydroquinone                            |                               | 0.2 g. |
|    | methylhydroquinone                             |                               | 0.2 g. |
|    | sodium sulfite                                 |                               | 0.9 g. |
|    | carboxymethylcellulose (sodium salt)           |                               | 44 g.  |
| 65 | Tamol SN <sup>®</sup> dispersant               |                               | 8.8 g. |
|    | carbon black                                   |                               | 172 g. |
|    | water to make 1 liter                          |                               |        |

## Processing Composition

### potassium hydroxide

The data in the following table are obtained by reflection densitometry after the elements had been laminated together for about 3 hr.

Table

| Temp.<br>°C. | Cover<br>Sheet | Sensitometric Comparisons |                           |                          | D <sub>min</sub><br>Red | D <sub>min</sub><br>Green | D <sub>max</sub><br>Blue |
|--------------|----------------|---------------------------|---------------------------|--------------------------|-------------------------|---------------------------|--------------------------|
|              |                | D <sub>max</sub><br>Red   | D <sub>max</sub><br>Green | D <sub>max</sub><br>Blue |                         |                           |                          |
| 15°          | A<br>(control) | 2.00                      | 1.89                      | 1.58                     | .28                     | .24                       | .23                      |
|              | B              | 2.08                      | 2.00                      | 1.60                     | .26                     | .22                       | .21                      |
| 22°          | A              | 2.22                      | 2.15                      | 1.85                     | .30                     | .28                       | .27                      |
|              | B              | 2.26                      | 2.20                      | 1.94                     | .30                     | .26                       | .25                      |
| 38°          | A              | 2.25                      | 2.16                      | 1.98                     | .46                     | .39                       | .33                      |
|              | B              | 2.25                      | 2.17                      | 1.97                     | .40                     | .30                       | .29                      |

The data show small but significant decreases in D<sub>min</sub> in all layers, particularly with high-temperature processing when a small amount of the blocked mercaptotetrazole derivative is incorporated in the cover sheet. At the lower temperatures a slight increase in D<sub>max</sub> also occurs.

Although the invention has been described in considerable detail with particular reference to certain preferred embodiments thereof, variations and modifications can be effected within the spirit and scope of the invention.

We claim:

1. A photographic element comprising a support and at least one layer thereon containing a silver halide emulsion having associated therewith a blocked development restrainer of the formula:



35

wherein Z represents the nonmetallic atoms necessary to form a nucleus which completes a 5- or 6-membered heterocyclic ring on said structure; R is a cyano group; and R<sup>1</sup> and R<sup>2</sup> can each be hydrogen atoms, alkyl groups or aryl groups, provided that at least one of R<sup>1</sup> and R<sup>2</sup> is a hydrogen atom.

2. A photographic element according to claim 1 wherein said R<sup>1</sup> and R<sup>2</sup> of said blocked development restrainer are hydrogen atoms.

3. A photographic element according to claim 1 wherein said blocked development restrainer has the formula:



50

4. A photographic element according to claim 1 wherein said blocked development restrainer has the formula:



60

wherein Z represents the nonmetallic atoms necessary to form a nucleus which completes a 5- or 6-membered ring and which, together with said sulfur atom, provides

a silver halide development restrainer upon cleavage from the remainder of the molecule.

5. A photographic element according to claim 1 wherein said layer containing a silver halide emulsion has at least 0.005 mole of said blocked development restrainer associated therewith per mole of silver in said layer.

6. A photographic element according to claim 1 wherein said silver halide emulsion is a negative silver halide emulsion.

7. A photographic element according to claim 1 wherein Z of said blocked development restrainer represents the atoms which form an uncharged tetrazole ring.

15

8. A photographic element according to claim 1 wherein aid layer containing said silver halide emulsion has associated therewith an image dye-providing material.

9. A photographic element according to claim 1 wherein said layer containing said silver halide emulsion has associated therewith an initially mobile, image dye-providing material.

10. A photographic element according to claim 1 wherein aid layer containing said silver halide emulsion has associated therewith a positive-working, initially immobile, image dye-providing material.

11. A photographic element comprising a support and at least one layer thereon containing a silver halide emulsion having associated therewith a blocked development restrainer of the formula:



35

40

12. A photographic element according to claim 11 wherein said silver halide emulsion is a negative silver halide emulsion.

13. A photographic element according to claim 11 wherein said layer containing said silver halide emulsion has associated therewith an image dye-providing material.

45

14. In an image-transfer film unit comprising:

50

a. a photosensitive element comprising a support having thereon at least one layer containing a silver halide emulsion having associated therewith an image dye-providing material,

b. an image-receiving layer and  
c. means containing an alkaline processing composition adapted to discharge its contents within said film unit,

55

the improvement wherein said silver halide emulsion has associated therewith a blocked development restrainer of the formula:



60

65

wherein Z represents the nonmetallic atoms necessary to form an uncharged nucleus which completes a 5- or 6-membered heterocyclic ring on said structure; R is a cyano group; and R<sup>1</sup> and R<sup>2</sup> can each be hydrogen

atoms, alkyl groups or aryl groups, provided at least one of  $R^1$  and  $R^2$  is a hydrogen atom.

15. A film unit according to claim 14 wherein said image-receiving layer is located on a separate support and is adapted to be superposed on said photosensitive element during processing.

**16.** A film unit according to claim 14 wherein said silver halide emulsion is a negative silver halide emulsion.

**17. A film unit according to claim 14 wherein said blocked development restrainer is located in said layer containing said silver halide emulsion.**

18. An image-transfer film unit adapted to be processed by passing said unit between a pair of juxtaposed pressure-applying members comprising:

- a. a photosensitive element comprising a support having thereon a layer containing a silver halide emulsion having associated therewith an image dye-providing material,
  - b. an image-receiving layer,
  - c. a cover sheet superposed or adapted to be superposed on said photosensitive element and
  - d. a means for discharging an alkaline processing composition within said film unit.

composition within said film unit, wherein at least one layer between said support and said cover sheet of said film unit contains a blocked 30 development restrainer having the formula:



wherein Z represents the nonmetallic atoms necessary to form a nucleus which completes a 5- or 6-membered heterocyclic ring on said structure; R is a cyano group; and R<sup>1</sup> and R<sup>2</sup> can each be hydrogen atoms, alkyl groups or aryl groups, provided at least one of R<sup>1</sup> and R<sup>2</sup> is a hydrogen atom.

19. A film unit according to claim 18 wherein said image-receiving layer is located on said cover sheet.

20. A film unit according to claim 18 wherein said support of said photosensitive element is a transparent support which has thereon said image-receiving layer, an opaque layer, a layer containing a red-sensitive silver halide emulsion, a layer containing a green-sensitive silver halide emulsion and a layer containing a blue-sensitive silver halide emulsion, at least one of said layers containing silver halide emulsion having associated therewith an image dye-providing material.

**21.** A film unit according to claim 20 wherein each of said layers containing silver halide emulsions has associated therewith an image dye-providing material.

22. A film unit according to claim 18 wherein said layer containing said silver halide emulsion has associated therewith at least 0.005 mole of said blocked development restrainer per mole of silver.

23. A film unit according to claim 18 wherein said blocked development restrainer is a compound having the formula:



24. A film unit according to claim 18 wherein said silver halide emulsion is a negative silver halide emulsion.

**25.** A film unit according to claim 23 wherein the cover sheet remains laminated with the photosensitive element after processing.

26. A film unit according to claim 18 wherein said  
15 image dye-providing material is an oxichromic devel-  
oper.

27. In a process for producing a photographic transfer image comprising:

- a. imagewise-exposing a photosensitive element comprising a support having thereon a layer containing a silver halide composition having associated therewith an image dye-providing material,
  - b. treating said photosensitive element with an alkaline processing composition to effect development of said exposed silver halide emulsion layer,
  - c. forming an imagewise distribution of diffusible image dye-providing material as a function of development of said silver halide emulsion layer, and
  - d. at least a portion of said imagewise distribution of diffusible image dye-providing material diffusing to an image-receiving layer.

the improvement wherein said silver halide emulsion has associated therewith a blocked development restrainer of the formula:



40 wherein Z represents the nonmetallic atoms necessary to form an uncharged nucleus which completes a 5- or 6-membered heterocyclic ring on said structure; R is a cyano group; and R<sup>1</sup> and R<sup>2</sup> can each be hydrogen atoms, alkyl groups or aryl groups.

45 28. A process according to claim 27 wherein said photosensitive element contains a layer containing a red-sensitive negative silver halide emulsion, a layer containing a green-sensitive negative silver halide emulsion and a layer containing a blue-sensitive negative silver halide emulsion, at least one of said layers containing silver halide emulsion having associated therewith an image dye-providing material.

29. A process according to claim 28 wherein each of  
said layers containing silver halide emulsions has asso-  
ciated therewith an initially diffusible image dye-prov-  
iding material.

30. A process according to claim 28 wherein each of said layers containing silver halide emulsions has associated therewith an initially immobile, image dye-producing material.

60 31. A process according to claim 27 wherein said photosensitive element is treated with an alkaline processing composition having a pH of at least 12.

32. A process according to claim 27 wherein said image dye-providing material is a positive-working, immobile, image dye-providing material.

33. A process according to claim 27 wherein said image dye-providing material is an oxichromic developer.

\* \* \* \* \*

UNITED STATES PATENT AND TRADEMARK OFFICE

CERTIFICATE OF CORRECTION

PATENT NO. : 4,009,029

Page 1 of 2

DATED : February 22, 1977

INVENTOR(S) : Hammond et al

It is certified that error appears in the above-identified patent and that said Letters Patent are hereby corrected as shown below:

Column 1, line 14, "photographic" should read --photographic--. Column 2, line 10, "particulaly" should read --particularly--; line 11, "about" should read --above--. Column 3, lines 23-24, "herterocyclic" should read --heterocyclic--. Column 4, line 6, "medium," should read --medium;--. Column 5, end of line 13, "in" should read --an--; line 67, "tyie" should read --type--. Column 6, line 58, "liguid" should read --liquid--. Column 10, line 37, that part of formula reading "cyanuethylthio)" should read -- cyanoethylthio)--; that part of formula reading "phenyltetrazale" should read --phenyltetrazole--. Column 11, line 29, that part of formula reading "disec" should read --di-sec--; line 37, that part of formula reading "disec" should read --di-sec--; line 46, that part of formula reading "disec" should read --di-sec--. Column 12, line 2, "4-metylphenyl" should read --4-methylphenyl--. Column 13, line 29, "photographic" should read --photographic--; lines 46-47, "2-cyanoethylthio)-lauramide" should read --diethyl lauramide--; line 47, that part of formula reading "(2:cyanoethylthio)" should read --(2-cyanoethylthio)--; line 51, "mg./ft.<sup>2</sup>, 5--" should read --mg./ft.<sup>2</sup>, 2,5--; line 52, "magenta" should read -- magenta--; line 60, that part of formula reading "tetrahydro5,8" should read --tetrahydro-5,8--; line 64, "diethyl" should read -- diethyl--; lines 66-67, "bromoidiode" should read --bromoiodide--. Column 15, line 63, that part of formula reading "secdodecylhydroquinone" should read --sec-dodecylhydroquinone--.

UNITED STATES PATENT AND TRADEMARK OFFICE  
CERTIFICATE OF CORRECTION

PATENT NO. : 4,009,029

DATED : February 22, 1977

INVENTOR(S) : Hammond et al

Page 2 of 2

It is certified that error appears in the above-identified patent and that said Letters Patent are hereby corrected as shown below:

Column 16, line 62, "various" should read --viscous--. Column 17, approximate line 27, "Dye Releaser I" should be placed further up the column with the compound structure to which it pertains. Column 18, line 4, "nd" should read --and--; line 65, that part of formula reading "secododecylhydroquinone" should read --sec-dodecylhydroquinone--. Column 20, lines 55-end, that part of formula set forth as:



should read



Column 23, line 41, "grup;" should read --group;--. Column 24, line 16, "aid" should read --said--; line 25, "aid" should read --said--; line 50, "therewtih" should read --therewith--.

Signed and Sealed this  
Seventeenth Day of May 1977

[SEAL]

Attest:

RUTH C. MASON  
*Attesting Officer*

C. MARSHALL DANN  
*Commissioner of Patents and Trademarks*